

## UNITED STATES PATENT OFFICE

2,273,831

## MAGNESIUM ALLOY

Arthur Burkhardt, Berlin - Lichterfelde, and Richard Knabe, Berlin-Zehlendorf, Germany, assignors to Georg Von Giesche's Erben, Breslau, Germany, a corporation of Germany

No Drawing. Application November 9, 1939, Serial No. 303,613. In Germany December 17, 1938

4 Claims. (Cl. 75—168)

Our invention relates to a magnesium alloy, and more especially to an alloy of the type described in U. S. Patent 2,159,964, for "Magnesium alloy," patented May 30, 1939.

In this patent, a magnesium alloy has been described that contains 2 to 6% bismuth, 0.5 to 3% cadmium, 1 to 5% aluminium, and 1 to 3.5% zinc. The remainder is substantially all magnesium. The phrase "substantially all magnesium" is intended to include magnesium and magnesium with minor amounts of customary impurities and auxiliaries. Such auxiliary alloying elements are, for instance, 0.1 to 2% each of manganese, calcium, silicon, or one of the metals of the iron group (iron, nickel, and cobalt) separately or collectively. Such and other auxiliaries are usual in magnesium alloys and they do not influence the characteristic properties of our novel alloys.

Investigations with alloys of the type described in the said U. S. patent have demonstrated that their properties can be improved by certain additions. Thus, it has been found that addition of silver at the rate of 0.1 to 5% is favorable.

According to our invention, magnesium alloys contain 2 to 6, preferably 4 to 5% bismuth, 0.5 to 3% cadmium, preferably about 2% cadmium, 1 to 5, preferably 2 to 4% aluminium, 1 to 3.5, preferably about 3% zinc, and about 0.1 to 5% silver, the remainder substantially all magnesium.

Silver-containing magnesium alloys have already been developed in England by the National Physical Laboratory, and magnesium alloys of high tensile strength have been produced by adding silver, but the ductility of these alloys is poor. For instance, a magnesium alloy containing aluminium and cadmium and 2% silver, has a tensile strength of 43 kg. per sq. mm. but its elongation is only 2%.

In contradistinction, alloys are obtained according to our invention, by adding silver to magnesium alloys as described in the said U. S. patent, which have 14 to 8% elongation and a tensile strength of 40 to 42 kg. per sq. mm.

Our novel silver-containing magnesium alloys are superior to those according to the said U. S. patent in that they can be heat treated due to the addition of silver, and that their workability is much improved. In the working of the alloys according to the said patent, it had been found that they do not work quite satisfactorily, and this drawback is eliminated by our invention. Furthermore, it has been found that in many

cases it is desirable to increase the zinc content of the alloys according to the said U. S. patent beyond 1 to 3.5%, and up to about 7%. In this manner the tensile strength is reduced slightly, viz., to 34 to 36 kg. per sq. mm. but the elongation rises to about 24 to 26%. Alloys of this kind are employed if maximum tensile strength is less important than high elongation.

Such an alloy according to the invention contains, in addition to the percentages of bismuth, cadmium, and aluminium indicated, 1 to 7% zinc and about 0.1 to 5% silver, remainder substantially all magnesium.

In the following tabulation, some examples of alloys according to our invention are given, it being understood that for all alloys in the tabulation the remainder is substantially all magnesium as defined above, that is, magnesium with or without the aforesaid minor amounts of customary impurities and/or auxiliaries.

## Examples

| No. | No. | Content of constituents, percent |    |    |    |     |
|-----|-----|----------------------------------|----|----|----|-----|
|     |     | Al                               | Bi | Cd | Zn | Ag  |
| 1   |     | 5                                | 4  | 2  | 3  | 0.5 |
| 2   |     | 5                                | 4  | 2  | 3  | 2   |
| 3   |     | 5                                | 2  | 3  | 3  | 1   |
| 4   |     | 5                                | 2  | 3  | 3  | 3   |
| 5   |     | 5                                | 4  | 2  | 5  | 0.8 |

We claim:

1. A light metal alloy containing 1 to 5% aluminium, 2 to 6% bismuth, 0.5 to 3% cadmium, from traces up to 7% zinc, from a small but effective amount up to 5% silver, and a remainder substantially all of magnesium with customary additions and impurities.
2. A light metal alloy containing 1 to 5% aluminium, 2 to 6% bismuth, 0.3 to 3% cadmium, 1 to 7% zinc, 0.1 to 5% silver, and a remainder substantially all of magnesium with customary additions and impurities.
3. A light metal alloy containing 2 to 4% aluminium, 4 to 5% bismuth, 0.5 to 3% cadmium, 1 to 3.5% zinc, 0.1 to 5% silver, and a remainder substantially all of magnesium with customary additions and impurities.
4. A light metal alloy containing about 2 to 4% aluminium, 4 to 5% bismuth, about 2% cadmium, about 3% zinc, 0.1 to 5% silver, and substantially all magnesium to make up 100%.

ARTHUR BURKHARDT.  
RICHARD KNABE.